

Nov. 15, 1938.

O. C. ROHDE

2,136,467

SPARK PLUG, INSULATING MATERIAL THEREFOR, AND METHOD OF MAKING THE SAME

Filed April 22, 1937

FIG. 1.



FIG. 2.



FIG. 3.



Inventor  
Otto C. Rohde

By

Conrad C. Rohde  
Witness

## UNITED STATES PATENT OFFICE

2,136,467

## SPARK PLUG, INSULATING MATERIAL THEREFOR, AND METHOD OF MAKING THE SAME

Otto C. Rohde, Toledo, Ohio, assignor to Champion Spark Plug Company, Toledo, Ohio, a corporation of Delaware

Application April 22, 1937, Serial No. 138,397  
In Canada May 16, 1936

19 Claims. (Cl. 123—169)

This application is a continuation in part of my prior application for "Spark plug", filed February 13, 1936, Serial No. 63,752.

This invention relates to a spark plug, and more particularly to a spark plug having a shell and a central electrode and powder compacted between the shell and electrode to form a seal, a holding means securing the parts in relative position, and insulation.

10 The invention further relates to an electric insulating material which is characterized by a high dielectric in combination with a relatively high conductivity of heat. The material is also impervious to gas and has a relatively high degree 15 of elasticity for material which is thus impervious.

The invention further relates to a method of producing the insulating material.

20 Details of the invention will appear as the description proceeds.

In the accompanying drawing forming a part of this specification,

Figure 1 is a longitudinal section of a spark plug embodying one form of the invention; Fig. 2 25 is a longitudinal section of a modified plug; Fig. 3 shows another modification of the plug, with a different shield.

30 In the form shown in Fig. 1, there is a conventional spark plug shell 10 provided with screw threads 11 adapting it to be screwed into the combustion chamber of an internal combustion motor. The shell has a central bore 12 provided near its inner end with a shoulder 13 on which rests an insulating ring 14 of mica or the like. 35 An electrode member 15 has its end 16 projecting into sparking relation with electrodes 17 mounted in the shell.

40 A conductor 18 of any suitable construction makes electrical contact with electrode 15 and extends outward to a connection 19 with a conductor 20 carried by an insulating member 21 on the inner end of a shield 22 which is secured to shell 10 by a threaded collar 23. The outer end 24 of conductor 20 extends into channel 25 45 of the shield and may be connected in any suitable manner to a conductor running through the shield.

Within bore 12 and above ring 14 there is a sleeve 26 threaded onto electrode 15 and resting 50 on ring 14. Around sleeve 26 and the lower end of conductor 18 there is compacted powder 27 which will be more fully described below.

Above the compacted powder 27 there is placed 55 an insulating member 28, which may be of porcelain or other suitable material. This may be

held in place by any suitable means. In the form illustrated a flange 29 of the shell is bent over and holds in place a washer 30 bearing upon the upper end of body 28. The parts are sufficiently held together by the compacted powder, but some means is desirable to prevent access of moisture to the compacted powder.

5 In the form shown in Fig. 2, many of the parts are identical, or substantially identical, with those shown in Fig. 1, and accordingly are given the same reference numerals and need not be separately described. The bore 12' of the shell shown in Fig. 3 is somewhat enlarged at its upper end, providing a shoulder 31 in addition to the shoulder 13'. Within this enlarged portion of the bore 15 there is the lower end of an insulating member 32, which may be of porcelain or an equivalent material, and which extends upward to connection 33. The electrode 15' is shown with an integral enlargement 34 in place of sleeve 26, and compacted material 27' surrounds this enlargement of electrode 15' in the same manner as described above, and also surrounds and holds in position the lower end of insulating member 32. The upper end of the compacted powder 27 may 25 be protected from moisture or the like by a washer 30' and inturned flange 29, similar to washer 30 and flange 29 described in connection with Fig. 1.

A conductor 18' of any suitable construction extends from electrode 15' to connection 33. 30 This conductor may be solid, hollow, or two-piece.

No shield is shown in Fig. 2, but it will be understood that any suitable shield may be attached, as by threads 35. 35

In Fig. 3 there is shown a modification in which no porcelain insulator is used. The parts similar to those shown in Fig. 1 are designated by similar reference characters.

The bore 12'' is made cylindrical above shoulder 13''. A conductor 36 extends from central electrode 15'' to connection 37. Around the outer end of conductor 36, and especially insulating it from washer 30'' and flange 29'', there is an insulating sleeve 38 of mica or the like. Between flange 29'' and connection 37 there are shown mica washers 39. A shield 40 with a lining 41 is shown screwed onto the shell 10'' by threads 35'.

The powder compacted at 27, 27', or 27'' may 50 be of the general type disclosed for sealing and holding purposes in my prior Patents Nos. 2,020,966 and 2,020,967, issued November 12, 1935. Mineral powder, that contains water of combination but is dry as to water of plasticity, 55

or free water, can in general be compacted by very heavy pressure to form a holding and sealing body; but lamellar crystalline mica and similar material which remains in scale-like particles, however finely ground, cannot be filled into and compacted uniformly in spaces like those commonly found in spark plugs, and therefore are not suitable for my purposes. Also, a material should be chosen which does not lose its water of combination at the temperature to which it is subjected in use.

Forming the powder into slip and spray-drying it into substantially spherical particles materially reduces the angle of repose and facilitates the ready and uniform filling of the powder into any space and consequently makes it feasible to compact the powder by high pressure in layers of suitable depth into a quite uniform material bonded throughout into a solid-gas-tight, slightly elastic body, having its particles in intimate holding contact with adjacent surfaces and with each other, so as to readily conduct heat.

In spray-drying the powder into spherical form, the fluidity of the slip, the manner of spraying, and the drying operation are so conducted that the surface tension of the liquid forms spherical drops of the sprayed slip, and retains these separated drops in substantially spherical form during the drying until the solid materials have been formed into substantially spherical shapes.

Where the material is to act as insulation, the basic compound should be chosen with regard to its inherent insulating character, and the resistance of such powder is greatly increased by treatment with a compound of the group consisting of boric acid and the borates of ammonium, magnesium, calcium, strontium and barium. Of these materials the borate of calcium is preferred as being very efficient and easily obtained. The borates of magnesium and barium are also quite effective and fairly easy to obtain. Strontium borate is not so readily available, and ammonium borate, while it has a distinctly beneficial effect, does not increase the dielectric to the extent that the other compounds mentioned will increase it.

A convenient way of treating the material with the boric compound is to dissolve the compound in the slip during its preparation for spray-drying. Not only does the compound increase the dielectric of the material, but it also makes the dried particles smoother and harder so that the dried material has a smaller angle of repose and pours and packs more readily, and it also reduces the tendency the material may have to be hygroscopic.

As indicated above, the materials should also be chosen in view of the heat to which the insulation will be subjected in use. For use as insulation in spark plugs where a considerable degree of heat is encountered, it has been found that materials of the class of ground soapstone or brucite or kaolin are useable, these materials being mentioned as readily available examples and not as an exhaustive list.

Such materials, properly prepared, form excellent insulation for spark plugs and similar purposes. For example, powdered talc formed into a slip with about 1% of calcium borate, then sprayed into fine drops and dried into substantially spherical pellets, can be compacted into an insulating body that has a much higher dielectric than ordinary porcelain insulating material, and at the same time has a conductivity

of heat of the order of that of iron or steel. Coupled with these qualities, it forms a gas-tight body and has sufficient resiliency to maintain this gas-tight joint in spite of frequent and sharp alterations in temperature, even when in contact with metallic members having materially different co-efficients of heat expansion. 5

It will be readily understood that, where insulation is to be employed in places not subjected to as high temperatures as spark plugs, 10 there is a wider range of choice of basic insulating powder, since there are many insulating crystalline materials having water of crystallization and satisfactory compacting characteristics, but which begin to lose water of crystallization 15 upon reaching the temperatures to which insulation is subjected in spark plugs.

While the construction of three forms of plug has been described and shown in some detail, it will be understood that many of the features may 20 be modified without departing from the invention as set forth in the appended claims, the chief feature of the invention being, as to the spark plug, the employment of the compacted powder 25 to perform the three functions of sealing, holding the parts in proper relation, and constituting an insulator.

While the compacted powder may be employed for substantially the full length of the shell, as shown in Fig. 1, it is particularly advantageous 30 at the inner end, where it is subjected to pressure of gases and to heat. At the outer end, which remains cooler, a body of any usual or suitable porcelain or the like may be used without incurring the leakage of gas or of electricity that 35 is likely to result at the inner end of a spark plug in a high compression, high duty motor.

While the insulating material described was developed primarily for spark plugs and has peculiar advantages when used for that purpose, it may 40 be employed for other uses where its qualities make it desirable, and therefore the broader of the appended claims directed to the insulating material are not confined beyond their stated terms to use in spark plugs or to material entirely suitable for such use. Substantially pure material is preferred, as generally having a higher dielectric, but some impurities are usually present in the commercial materials, and for many purposes considerable mixtures of less perfect insulating material is permissible. 45

The condition of the powder when compacted so that its grains interlock to form a good insulating gas-tight body gripping the adjacent parts and holding them in their desired relation, may 55 be termed "conglomerated", to distinguish from powder, such as most anhydrous rock powder, that remains separate particles in spite of any readily available amount of pressure, and from compactible powder that is not subjected to the 60 kind or degree of compacting that results in the described body of interlocked particles.

What I claim is:

1. A spark plug comprising a shell of conducting material, a central electrode, a body of 65 compacted and conglomerated powder between the shell and electrode, having interlocking particles forming a gas-tight joint, holding the shell and electrode in their desired relative positions, and constituting, for at least a portion of 70 the length of the shell, the sole insulation between the shell and electrode, and means protecting the ends of the body of compacted powder from moisture.

2. A spark plug comprising a shell of conduct- 75

ing material, a central electrode, and insulation between the shell and electrode, the outer portion of the insulation comprising a porcelain insulating body and the sole insulation between the 5 electrode and shell near the inner end of said insulation consisting of compacted and conglomerated powder having interlocking particles forming a gas-tight joint and the conglomerated powder holding in the shell, electrode and porcelain 10 material in their assembled relative positions.

3. A spark plug comprising a shell of conducting material, a central electrode, and a body of compacted and conglomerated powder, consisting 15 chiefly of magnesium silicate, between the shell and electrode, having interlocking particles forming a gas-tight joint, holding the shell and electrode in their desired relative positions, and constituting, for at least a portion of the length 20 of the shell, the sole insulation between the shell and electrode.

4. A spark plug comprising a shell of conducting material, a central electrode, and insulation between the shell and electrode, the insulation, 25 for at least a portion of its length, consisting of compacted and conglomerated powdered insulating crystalline material containing water of crystallization, that is not lost at the temperature to which it is subjected in use, and treated with a 30 compound of the group consisting of boric acid and the borates of ammonium, magnesium, calcium, strontium and barium.

5. A spark plug comprising a shell of conducting material, a central electrode, and insulating 35 material between the shell and electrode, the insulation, for at least a portion of its length, consisting of compacted and conglomerated magnesium silicate treated with calcium borate.

6. A spark plug comprising a shell of conducting material, a central electrode, and insulating 40 material between the shell and electrode, the insulation, for at least a portion of its length, consisting of compacted and conglomerated spray-dried pellets of magnesium silicate with a small 45 amount of calcium borate.

7. An insulating body consisting essentially of compacted insulating crystalline powder containing water of crystallization and treated with a 50 compound of the group consisting of boric acid and the borates of ammonium, magnesium, calcium, strontium and barium.

8. An insulating body consisting of magnesium silicate treated with calcium borate.

9. A material for use in electric apparatus consisting of a powder formed of approximately 55 spherical particles composed principally of in-

sulating crystalline material containing water of crystallization and impregnated with a material of the group consisting of boric acid and the borates of ammonium, magnesium, strontium and barium. 5

10. A material in accordance with claim 9 and in which the principal ingredient is magnesium silicate.

11. A material in accordance with claim 9 and in which the principal ingredient is brucite. 10

12. A material in accordance with claim 9 and in which the principal ingredient is kaolin.

13. Electric insulation consisting of compacted pellets made by spray-drying a slip of magnesium silicate containing a small amount of calcium 15 borate.

14. Insulating material consisting of spray-dried pellets of magnesium silicate with a small amount of calcium borate.

15. The method of preparing material for use 20 in electric apparatus which consists in forming a slip containing as its major ingredient finely ground crystalline insulating material containing water of crystallization, said slip also having dissolved therein a compound of the group consisting of boric acid and the borates of ammonium, magnesium, calcium, strontium and barium, spraying said slip into separated drops under conditions which cause the drops to assume spherical form and drying the separated drops in 30 approximately spherical form.

16. A method in accordance with claim 15 in which the principal ingredient of the slip is magnesium silicate.

17. A method in accordance with claim 15 and 35 in which the principal ingredient of the slip is brucite.

18. A method in accordance with claim 15 in which the principal ingredient of the slip is kaolin. 40

19. A method of forming electric insulation which comprises forming a slip containing as its major ingredient finely ground crystalline insulating material containing water of crystallization, said slip also having dissolved therein a compound of the group consisting of boric acid and the borates of ammonium, magnesium, calcium, strontium and barium, spraying said slip into separated drops under conditions which cause the drops to assume spherical form, drying the separated drops in approximately spherical form, and compacting the spherical particles into a unitary gas-tight elastic mass having a high 45 dielectric and high thermal conductivity. 50

OTTO C. ROHDE. 55